

## UNITED STATES PATENT OFFICE.

BURNHAM E. FIELD, OF DOUGLASTON, AND RUSSELL FRANKS, OF ELMHURST, NEW YORK, ASSIGNORS TO HAYNES STELLITE COMPANY, A CORPORATION OF INDIANA.

## WEAR-RESISTING ALLOY.

No Drawing.

Application filed December 24, 1925. Serial No. 77,575.

The invention is an alloy useful as a material for making articles subject to abrasive wear, such as bearings and gages, and for other purposes.

5 The alloy comprises as its essential constituents tungsten, chromium, carbon, boron and iron; and silicon is a valuable constituent though not strictly essential. The tungsten content is preferably between 1 per cent and 12 per cent; the chromium between 25 per cent and 35 per cent; the carbon between 1.0 and 3.5 per cent and the boron between 0.1 and 1.0 per cent; with the remainder principally iron. Silicon is usually 10 present in such metals and alloys as are used in preparing the alloy of the invention and is therefore a normal constituent of the final alloy. In many cases it is advantageous to increase the silicon content beyond the value 15 at which the fortuitous sources of silicon referred to would fix it: for example to bring the total silicon content to between 1.0 and 3.0 per cent. Manganese also enters the alloy in small quantities as a minor constituent of the raw materials, and manganese may be intentionally added as a deoxidizer. Various other metals and metalloids 20 may be present in small amounts, as is the case with the majority of alloys.

25 The hardness of the alloy increases as the tungsten and carbon are increased within the range given, while diminishing the contents of these elements increases toughness. Boron imparts strength and improves the 30 grain structure and silicon to a decidedly less degree has a somewhat similar action. Either of these elements if its proportion is unduly increased causes the alloy to become too brittle for the use contemplated.

35 It will be obvious that since each of the elements mentioned has a tendency to produce brittleness if increased to its upper limit, a proper balance between hardness and toughness will not be obtained by simultaneously using all of the elements in maximum quantity.

A composition which is excellent for many purposes contains tungsten about 7.5 per cent; chromium about 30 per cent; boron

about 0.4 per cent; carbon 2.5 to 3.0 per cent; and silicon 1.0 to 1.5 per cent. A specific alloy of about this composition contained:

|    | Per cent. |    |
|----|-----------|----|
| W  | 7.11      | 55 |
| Cr | 29.53     |    |
| B  | 0.39      |    |
| C  | 3.05      |    |
| Si | 1.50      |    |
| Mn | 0.39      | 60 |

The Brinell hardness of cast bars of this alloy was 512 and the scleroscope hardness 64. The breaking strength in transverse of one-half inch square cast bars held cantilever fashion with the load applied one inch 65 from the support was 2360 pounds.

The alloy may be made by melting together commercial metals and alloys containing suitable proportions of the elements desired in the final alloy, and no particular difficulty will be encountered in its preparation. The materials may be, for example, ferro-chromium and ferro-tungsten of suitable carbon content and a boron compound 70 or alloy such as boron-carbide, manganese-boron or chromium-boron. Approximately one-half of the boron added to the charge is recovered in the final alloy. Within the preferred range given the alloy is not readily forgeable or machinable. It can be cast 75 without difficulty to the desired shape and finished by grinding. No heat treatment is necessary as the hardness of the alloy is developed at the time of solidification.

## We claim:

1. A ferrous alloy suitable for making articles subject to abrasion, containing tungsten 1 to 12 per cent; chromium 25 to 35 per cent; boron 0.10 to 1.0 per cent; and carbon 1 to 3.5 per cent.

2. A ferrous alloy suitable for making articles subject to abrasion containing, approximately: tungsten 7.5 per cent; chromium 30 per cent; boron 0.4 per cent; carbon 2.5 to 3.0 per cent; and silicon 1.0 to 1.5 per cent.

3. An article of manufacture designed for a use wherein it is subject to abrasion

composed of an alloy containing tungsten 1 to 12 per cent; chromium 25 to 35 per cent; boron 0.10 to 1.0 per cent; and carbon 1 to 3.5 per cent.

- 5 4. An article of manufacture designed for a use wherein it is subject to abrasion composed of an alloy containing, approximately:

tungsten 7.5 per cent; chromium 30 per cent; boron 0.4 per cent; carbon 2.5 to 3.0 per cent; and silicon 1.0 to 1.5 per cent.

In testimony whereof, we affix our signatures.

BURNHAM E. FIELD.  
RUSSELL FRANKS.